

April 19, 1938.

A. POTT

2,114,456

METHOD OF PREPARING A POWDERED CARBONACEOUS MATERIAL FOR COMBUSTION ENGINES

Filed April 5, 1935



INVENTOR  
ALFRED POTT

BY  
*John J. Speckenbauer*  
ATTORNEY

## UNITED STATES PATENT OFFICE

2,114,456

## METHOD OF PREPARING A POWDERED CARBONACEOUS MATERIAL FOR COMBUSTION ENGINES

Alfred Pott, Essen-on-the-Ruhr, Germany

Application April 5, 1935, Serial No. 14,793  
In Germany October 17, 1934

6 Claims. (Cl. 44—1)

This invention relates to a method of preparing carbonaceous powdered fuel material for combustion engines, particularly those of the Diesel type. In such engines, air for combustion is compressed and thereby heated to such an extent that the fuel is automatically ignited at the desired moment. To this effect, in engines using liquid fuel, the latter is introduced into the highly compressed and very hot air by means 5 of a stream of more highly compressed air. In engines provided with pistons, the liquid fuel is thus injected just before the piston approaches the end of its stroke of compression. In engines to be fed with powdered solid fuel material, however, difficulties have been experienced when the fuel was simply injected. No complete combustion of the fuel which apparently does not ignite as readily as liquid fuel could be obtained; among other reasons this may be to its relatively 10 larger size and heat capacity and its relatively smaller active surface compared with finest drops of liquid fuel. Therefore, it is advisable to introduce the powdered carbonaceous material into the combustion air in ample time before 15 the temperature of ignition is reached, in order to permit the fuel to be thoroughly heated.

In such engines another difficulty has been encountered due to the ash content in the fuel material. Ashes in amounts sufficient to grind 20 off the cylinder and piston surfaces remain in the machine after combustion. The lubricating oil circulating in the machine transports the ash to other sensitive parts of the machine, resulting in considerable wear within a short time of 25 operation.

It is an object of the invention to present a carbonaceous powdered fuel material in a state of high purity, practically free from ash.

It is a further object of the invention to present the powdered carbonaceous fuel material in a state of high activity.

It is still another object of the invention to render the combustion, calculated upon the original solid fuel material, very effective.

According to the invention, no natural carbonaceous powdered material but solid powdered extracts of such material is used as fuel. Due to their production, such extracts are free or freed of ash and other impurities to any desired degree, therefore, not leaving in the machine any detrimental residues. Furthermore, the extracts being practically pure carbon substance and forming depolymerized and slightly hydrogenated products, such extracts are more active than 55 the initial coal substance, all the more so be-

cause of the absence not only of incombustible material but of constituents which tend to increase the fuel's heat capacity as well.

Various processes of manufacturing such extracts of coal, lignite, peat, etc. are known, using organic solvent media at elevated temperatures and, preferably, raised pressure during extraction. All these extracts of coal, lignite, etc. may be used for the purposes of the invention provided they are sufficiently free or freed of incombustible residues. If the normal purity of the extracts is still insufficient, filtration has to be effected preferably under raised pressure and at highly elevated temperatures.

Furthermore, in order to obtain great efficiency of the original fuel material, high yields of extracts are imperative. For this purpose, the invention uses a method of producing the extracts based on the following observation. If e. g. coal is treated in an autoclave with a suitable solvent medium, such as a mixture of lower and higher boiling oils, thereby gradually raising the temperature and registering the rising pressure in the autoclave by means of an indicator, a sudden increase of pressure can be observed at a certain temperature. This is due to the fact that a decomposition of the material under treatment takes place whereby gases are evolved. Therefore, if the temperature at a subsequent treatment of material of the same kind, with the same solvent media, remains a few degrees centigrade below the temperature of decomposition, so established by a previous treatment, a certain yield of extracts can be obtained. However, no matter how long such treatment at this temperature might be extended, or how often it might be repeated, the yield of extracts does not materially increase. After having obtained a first yield of extracts in the way described, the temperature of treatment may be raised, however, without causing decomposition, i. e. the evolving of gases indicated by suddenly increasing pressure. By the first treatment all the constituents capable of decomposition at the first established temperature are extracted from the carbonaceous material and taken in solution by the solvent medium, which protects them against further decomposition, and a balance of solid carbonaceous material remains the constituents of which are incapable of decomposition at this temperature. If, however, the temperature is gradually raised above the first mentioned level, a temperature will again be reached at which decomposition, indicated by a sudden rise of pressure, reoccurs. Therefore, a

second extraction has to be effected at a temperature above the first extraction temperature but by a few degrees centigrade lower than the second, higher temperature of decomposition established in the way described. Surprisingly, in this second stage in which the balance of the solid carbonaceous material is being treated at a temperature higher than the first one, a new substantial yield of extracts will be obtained in addition to that obtained during the first treatment. In continuing this procedure, one may cautiously raise the temperature more and more, obtaining thereby additional yields of extracts until a temperature has been reached at which the last yield of extracts is achieved and no additional amounts of extracts are obtainable, neither by repeating nor by extending the heat treatment at the last and highest temperature nor by further raising this temperature. In the latter case neither a decomposition can be observed (no sudden increase of pressure occurs any more) nor will additional extracts result. This last temperature depends upon the composition of the carbonaceous material under treatment, and this and all the foregoing temperatures of treatment, which are close to but below the decomposition temperature of the carbonaceous material under treatment, are to be established for every individual material in the way described hereinbefore.

If but a small amount of gases is evolved thereby and depending upon the nature of the material, the treatment may also be performed at about the various decomposition temperatures, provided the decomposition of a small part of the constituents is of no consequence.

From this it results that the extraction may be effected at elevated temperatures which are step-wise or gradually raised so that they are close to the decomposition temperature of the solid carbonaceous material under treatment and increased with the increasing amount of substance extracted from the material and taken in solution by the solvent media used. The pressure under which the treatment is performed is usually the normal pressure originating at the temperature applied for the treatment performed in a closed vessel (autoclave). Additional pressure may be applied, however.

As solvent media, among others, hydrogenated and/or acidic organic oils, alone or in mixture, may be used. By way of example only, a mixture of 40 parts naphthalene, 40 parts tetraline and 20 parts of a tar phenol boiling at about 230° C., or a mixture of tetraline and phenols in a ratio of e. g. 1:1, or anthracene oil alone, or in mixture with phenols or other oils such as tetraline or benzole, may be used.

In the drawing, a diagram is shown for the treatment of a long-flaming coal with a solvent medium consisting of 40 parts naphthalene, 40 parts tetraline and 20 parts tar phenols obtained by distillation of coal between 180° to 230° C. The long-flaming coal has been powdered or suitably broken up and then mixed with the solvent medium. The amount of solvent medium applied depends upon its nature and that of the carbonaceous material to be extracted. The weight of the solvent medium may be, for instance, equal to that of the carbonaceous material, or it may be higher or lower.

The coal and the solvent are deposited into an autoclave provided with a stirring device and treated therein for about three to four hours.

It has been established by special experiments

with this coal that a first decomposition occurs at 330° C. The constituents decomposing at about this temperature having been extracted, the remaining solid carbonaceous material decomposes a second time at 360° C., whereupon after additional extracts have been made at this second temperature range a third, fourth and fifth decomposition temperature occurs at about 380°, 400° and 410° C., respectively. Therefore, as the diagram shows, the coal had been heated up to 330° C. when the first extracts were made which may remain in the solvent medium or may be removed from it. Thereupon the temperature has been gradually or stepwise increased up to 410° to 415° C., and a second, third, fourth and fifth extract were obtained at about 360°, 380°, 400° and 410° to 415° C., respectively. As shown in the diagram, no additional extracts could be obtained at the sixth and seventh extraction, and therefore further raising of the temperature or continuation of the treatment at about 410° C. is ineffective. The pressure in the autoclave was ultimately raised to about 70 to 90 atmospheres. No destruction of the solvent medium took place because of this increased pressure in spite of the temperature being substantially above the normal boiling temperature under atmospheric pressure of some parts of the solvent media. Calculated upon the weight of the original, not disintegrated coal material, by the first extraction about 37% extracts were obtained, by the second extraction additional 8%, with additional yields at further extractions so that the entire yield of extracts amounted to about 74%. The remaining solid material consisted of coke and ash not capable of further disintegration. As a matter of fact, depending upon the nature of the coal under treatment, yields up to 94% may be obtained in this way. Thus, any and all combustible constituents are extracted from the fuel material, and the highest efficiency is achieved as far as the given solid fuel material is concerned.

The extracts so obtained are highly active. The extracts being solid at normal temperature up to about 200° C. and over, coal extracts up to about 230° to 250° C., they can be conveniently separated from the solvents by gradually cooling the solvents still containing the dissolved extracts.

If some undesired amounts of ash and other not disintegrated parts of the carbonaceous material remain in the extracts, they may be separated by centrifugation or filtration or by allowing the solution to stand so that the heavier solid particles may precipitate. If, due to the extremely fine dispersion of the impurities referred to none of these methods succeeds, then the extracts still dissolved in the solvent medium may be filtered under raised pressure and at highly elevated temperature. Thereby practically pure extracts are obtained, the content of undesirable solid particles being substantially below 1% and, as a great number of investigations have proven, amounting to only a few tenths of one per cent down to less than one tenth of one per cent. For this filtration any suitable filter and filter material may be used. The solid residue of extraction of carbonaceous material is most suitable as filter material for the extracts obtained therefrom. As average temperatures for this filtering 150° to 170° C., may be mentioned, but higher or lower temperatures may be applied. As the lowest limit a temperature range of about 75° to 100° C. may be given. The pressure may be chosen above about 5 atmos-

phers per square centimeter and very good results have been obtained within the range of 10 to 20 atmospheres. In this way extracts are obtained which are both easily and fully combustible and extremely pure.

These extracts being solid at normal and elevated temperatures up to certain limits mentioned above, are now to be powdered in any suitable way and to any desired fineness. Ball mills may be used and the treatment therein extended sufficiently long to obtain the desired size of powder.

As an engine suitable for the powdered carbonaceous extract according to the invention the motor described in the periodical "Oel und Kohle", December 1933, pages 135, 136, may be referred to. This motor uses an additional chamber in which measured quantities of powdered solid fuel are delivered ahead of each compression stroke of the piston. The chamber is in open connection with the cylinder so that the compressed and heated air enters this chamber and gradually heats the fuel deposited therein until its ignition starts automatically and the evolved gases of combustion expand into the cylinder, injecting into it simultaneously the still burning fuel.

It is to be understood, however, that the invention is not limited to the use of this or any other type of a reciprocating or continuously turning engine adapted to be operated with powdered solid fuel material.

It is further to be understood that the fuel material according to the invention may be used as such alone or in admixture to any other powdered solid or even liquid fuel material.

In the appended claims the term "solvent" comprises any suitable solvent medium for the constituents to be extracted, or any mixture of such solvent media.

What I claim is:

1. A carbonaceous fuel material for combustion engines consisting substantially of powdered solid extracts obtained from solid carbonaceous material by treating it in closed vessels with solvents at gradually increasing temperatures and correspondingly rising pressures, said temperatures lying close to the increasing temperatures of decomposition of the carbonaceous material under treatment and raised until no additional yields of extracts are obtained, said extracts separated from the solid residues and powdered.

2. A carbonaceous fuel material for combustion engines consisting substantially of powdered solid extracts obtained from solid carbonaceous material by treating it in closed vessels with solvents at stepwise increasing temperatures and correspondingly rising pressures, said temperatures lying close to the increasing temperatures

of decomposition of the carbonaceous material under treatment and raised until no additional yields of extracts are obtained, said extracts separated from the solid residues and powdered.

3. A carbonaceous fuel material for combustion engines consisting substantially of powdered solid extracts obtained from solid carbonaceous material by treating it in closed vessels with solvents at gradually increasing temperatures and correspondingly rising pressures, said temperatures lying close to the increasing temperatures of decomposition of the carbonaceous material under treatment and raised until no additional yields of extracts are obtained, said extracts separated from the solid residues by filtration under elevated temperatures above about 75° C. and under raised pressure above about 5 atmospheres per sq. cm., and thereupon powdered.

4. A carbonaceous fuel material for combustion engines consisting substantially of powdered solid extracts obtained from solid carbonaceous material by treating it in closed vessels with solvents at stepwise increasing temperatures and correspondingly rising pressures, said temperatures lying close to the increasing temperatures of decomposition of the carbonaceous material under treatment and raised until no additional yields of extracts are obtained, said extracts separated from the solid residues by filtration under elevated temperatures above about 75° C., and under raised pressure above about 5 atmospheres per sq. cm., and thereupon powdered.

5. A method of producing carbonaceous fuel material for combustion engines comprising the steps of extracting solid carbonaceous material with solvents in closed vessels at increasing temperatures and correspondingly rising pressures, said temperatures lying close to the increasing temperatures of decomposition of said carbonaceous material, and raised until no additional yields of extracts are obtained, separating the extracts thus obtained from the solid residues of said material, allowing said extracts to solidify, and thereupon powdering said solid extracts.

6. A method of producing carbonaceous fuel material for combustion engines comprising the steps of extracting solid carbonaceous material with solvents in closed vessels at increasing temperatures lying close to the increasing temperatures of decomposition of said carbonaceous material, and raised until no additional yields of extracts are obtained, separating the extracts thus obtained from the solid residues of said material by means of filtration at elevated temperatures above about 75° C. and raised pressure above about 5 atmospheres per sq. cm., allowing said extracts to solidify, and thereupon powdering said solid extracts.

ALFRED POTT.